

## UNITED STATES PATENT OFFICE

2,076,153

## LUBRICATING OIL

Francis J. Licata, New York, N. Y., assignor to  
 National Oil Products Company, Harrison, N. J.,  
 a corporation of New Jersey

No Drawing. Application March 1, 1933, Serial  
 No. 659,175

## 6 Claims. (Cl. 87-9)

My invention relates to lubricating oils and refers particularly to means for reducing the congealing point, or pour point, of lubricating oils.

When a lubricating oil, containing paraffin, or other waxes, or substances having a higher congealing, or pouring, point than the oil itself, is cooled, the wax, or other substances begins to separate from the oil, and if the temperature is low enough the oil flows with difficulty or ceases to flow.

It is desirable that a lubricating oil should remain fluid at all stages of employment from the starting of the engine to its full operation.

It is also desirable that the oil should remain fluid at all ordinary temperatures of use, and that it should not become thick, congealed or slow to flow at winter temperatures.

Attempts have been made to accomplish these desirable results by dewaxing, or removing, the wax from the oil by means of abnormal low temperatures, cold settling, solvents, centrifuging, etc., but all of these methods are accompanied by considerable expense, and time, and require considerable apparatus for their accomplishment.

I have found that it is not necessary to remove the waxes from the oil in order to obtain the desired low pour point, but that this result can be obtained by adding a small amount of diethylene-glycol to the oil.

When diethylene-glycol is mixed with a mineral lubricating oil, the two ingredients have a tendency to separate upon standing, thus preventing a constant uniform mixture and decreasing the value of the mixture for lubricating purposes.

In order to overcome this objectionable feature, I employ an aluminum soap, such as aluminum stearate, aluminum oleate, or aluminum naphthenate, which has the property of retaining the diethylene-glycol uniformly throughout the oil.

While a mixture of diethylene-glycol and an aluminum soap may be successfully employed for the accomplishment of the described results, I have found that for certain classes of lubricating oils, it is advisable to include a substance which will render the oil less viscous and hence freer flowing, and among such substances, which for purposes of identification in my invention I call "de-viscosizing substances", are the ricinoleic fatty acids, the higher fatty alcohols, latex and paraffin oil; and my invention relates to the employment of diethylene-glycol and an aluminum soap, both with and without a de-viscosizing substance.

I give the following as examples of my invention:

## Example 1

A mixture is made of:

|                        | Percent |
|------------------------|---------|
| Diethylene-glycol      | 15      |
| Castor oil fatty acids | 15      |
| Aluminum stearate      | 70      |

When  $\frac{1}{2}\%$  of the above mixture is added to a S. A. E. 30 oil, the pour point is lowered from 10° F. to  $-15^{\circ}$  F. When the same quantity is added to a S. A. E. 50 oil, the pour point is lowered from 15° F. to  $-10^{\circ}$  F.

## Example 2

A mixture is made of:

|                   | Percent |
|-------------------|---------|
| Diethylene-glycol | 2       |
| Latex             | 15      |
| Aluminum stearate | 83      |

and added to a lubricating oil.

## Example 3

A mixture is made of:

|                     | Percent |
|---------------------|---------|
| Diethylene-glycol   | 7       |
| Paraffin oil 28° F. | 80      |
| Aluminum oleate     | 13      |

and added to a lubricating oil.

## Example 4

A mixture is made of:

|                   | Percent |
|-------------------|---------|
| Diethylene-glycol | 15      |
| Aluminum stearate | 85      |

and added to a lubricating oil.

It will thus be seen that I can thus lower the pour point of the oil, thus greatly enhancing its value and efficiency without the expense incident to the actual physical removal of the wax, and similar substances, from the oil.

I do not limit myself to the particular oils, chemicals, times, quantities and steps of procedure particularly mentioned, as these are used simply as a means for clearly explaining my invention.

## What I claim is:

1. A non-water-dispersible, wax-containing, petroleum lubricating oil containing diethylene-glycol, castor oil fatty acids and an aluminum soap.
2. A non-water-dispersible, wax-containing, petroleum lubricating oil containing diethylene-glycol, castor oil fatty acids and aluminum stearate.

55

3. A mixture adapted for reducing the pour point of non-water-dispersible, wax containing, petroleum lubricating oil consisting of diethylene-glycol, a de-viscosizing substance of the group consisting of ricinoleic acid, the higher fatty alcohols and paraffin oil, and an aluminum soap.

4. A mixture adapted for reducing the pour point of non-water-dispersible, wax containing, petroleum lubricating oil consisting of diethylene-glycol, a de-viscosizing substance of the group consisting of ricinoleic acid, the higher fatty alcohols and paraffin oil, and aluminum stearate.

5. A mixture adapted for reducing the pour point of non-water-dispersible, wax containing, petroleum lubricating oil consisting of diethylene-glycol, castor oil fatty acids and an aluminum soap.

6. A mixture adapted for reducing the pour point of non-water-dispersible, wax containing, petroleum lubricating oil consisting of diethylene-glycol, castor oil fatty acids and aluminum stearate.

5

10

FRANCIS J. LICATA.